



US011608551B2

(12) **United States Patent**  
**Lin et al.**

(10) **Patent No.:** US 11,608,551 B2  
(45) **Date of Patent:** Mar. 21, 2023

(54) **ALUMINUM ALLOYS, AND METHODS FOR PRODUCING THE SAME**

(71) Applicant: **HOWMET AEROSPACE INC.**, Pittsburgh, PA (US)

(72) Inventors: **Jen C. Lin**, Export, PA (US); **Gabriele F. Ciccola**, Hudson, OH (US); **Santosh Prasad**, Murrysville, PA (US); **Wei Wen**, Allison Park, PA (US); **Raymond J. Kilmer**, Pittsburgh, PA (US)

(73) Assignee: **Howmet Aerospace Inc.**, Pittsburgh, PA (US)

(\*) Notice: Subject to any disclaimer, the term of this patent is extended or adjusted under 35 U.S.C. 154(b) by 323 days.

(21) Appl. No.: **16/848,656**

(22) Filed: **Apr. 14, 2020**

(65) **Prior Publication Data**

US 2020/0277691 A1 Sep. 3, 2020

**Related U.S. Application Data**

(63) Continuation of application No. PCT/US2018/058421, filed on Oct. 31, 2018.  
(Continued)

(51) **Int. Cl.**  
**C22F 1/057** (2006.01)  
**C22C 21/02** (2006.01)

(Continued)

(52) **U.S. Cl.**  
CPC ..... **C22F 1/057** (2013.01); **C22C 21/02** (2013.01); **C22C 21/10** (2013.01); **C22C 21/14** (2013.01);  
(Continued)

(58) **Field of Classification Search**  
CPC ..... C22F 1/002; C22F 1/043; C22F 1/053;  
C22F 1/057; C22C 21/02; C22C 21/08;  
(Continued)

(56) **References Cited**

U.S. PATENT DOCUMENTS

|              |         |               |
|--------------|---------|---------------|
| 5,888,320 A  | 3/1999  | Dorward       |
| 6,132,531 A  | 10/2000 | Fang et al.   |
| 6,317,913 B1 | 11/2001 | Kilmer et al. |
| 6,344,237 B1 | 2/2002  | Kilmer et al. |

(Continued)

FOREIGN PATENT DOCUMENTS

|               |   |        |
|---------------|---|--------|
| JP 10219381 A | * | 8/1998 |
| JP H10-219381 |   | 8/1998 |

(Continued)

OTHER PUBLICATIONS

B. Raeisinia et al. "Examination of precipitation in the aluminum alloy AA6111 using electrical resistivity measurements" Materials Science and Engineering A 420 (2006) 245-249. (Year: 2006).\*

(Continued)

*Primary Examiner* — Anthony J Zimmer

*Assistant Examiner* — Nazmun Nahar Shams

(74) *Attorney, Agent, or Firm* — Greenberg Traurig, LLP

(57) **ABSTRACT**

New aluminum alloys are disclosed and generally include 0.6-1.4 wt. % Si, 0.25-0.90 wt. % Mg, wherein the ratio of wt. % Si to wt. % Mg is from 1.05:1 to 5.0:1, 0.25-2.0 wt. % Cu, 0.10-3.5 wt. % Zn, 0.01-1.0 wt. % Fe, up to 0.8 wt. % Mn, up to 0.25 wt. % Cr, up to 0.20 wt. % Zr, up to 0.20 wt. % V, and up to 0.15 wt. % Ti, wherein the total of Fe+Mn+Cr+Zr+V+Ti is not greater than 2.0 wt. %, the balance being aluminum and impurities. The new aluminum alloys may include Q phase precipitates. In some embodiments, the solvus temperature of the Q phase precipitates is not greater than 950° F.

**13 Claims, 2 Drawing Sheets**



**Related U.S. Application Data**

|      |                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                         |                                                                                                                                                                                                                                                                                                                                                                                                                                                                                                                                                                                                                                                                                                                                                                                                                                                                                                                                                                                                                                                                                   |                                                                                                                                                                                                                                                                                                                                                                                                                                                                                                                                                                                                                                                                                                                                                                                                                                                                                                                                                                                                                                                                                                                                                                                       |
|------|---------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|-----------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|---------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| (60) | Provisional application No. 62/715,163, filed on Aug. 6, 2018, provisional application No. 62/579,728, filed on Oct. 31, 2017.                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                          | 2005/0095447 A1<br>2005/0167012 A1<br>2005/0238528 A1<br>2006/0078728 A1<br>2006/0289093 A1<br>2007/0125460 A1<br>2008/0066833 A1<br>2008/0274367 A1<br>2010/0047113 A1<br>2010/0089503 A1<br>2010/0129683 A1<br>2010/0276108 A1<br>2010/0304175 A1<br>2011/0247736 A1<br>2012/0055590 A1<br>2012/0156089 A1<br>2014/0166165 A1<br>2014/0230974 A1<br>2014/0366997 A1<br>2014/0366998 A1<br>2014/0367000 A1<br>2015/0020930 A1<br>2015/0217599 A1<br>2016/0107265 A1<br>2016/0160333 A1<br>2017/0009325 A1<br>2017/0014937 A1<br>2017/0088920 A1<br>2017/0120386 A1<br>2017/0120393 A1<br>2017/0121795 A1<br>2017/0175239 A1<br>2017/0175240 A1<br>2017/0292174 A1<br>2017/0306447 A1<br>2017/0306448 A1<br>2017/0306449 A1<br>2017/0306450 A1<br>2017/0306457 A1<br>2017/0306460 A1<br>2017/0314112 A1<br>2017/0326690 A1<br>2017/0326868 A1<br>2017/0369978 A1<br>2018/0171438 A1<br>2018/0179621 A1<br>2018/0200834 A1<br>2019/0193149 A1<br>2019/0193158 A1<br>2019/0309402 A1<br>2019/0357647 A1<br>2020/0056268 A1<br>2020/0080182 A1<br>2020/0115780 A1<br>2020/0189314 A1 | 5/2005 Baumann et al.<br>8/2005 Lin et al.<br>10/2005 Lin et al.<br>4/2006 Kilmer<br>12/2006 Yan et al.<br>6/2007 Lin et al.<br>3/2008 Lin et al.<br>11/2008 Kilmer et al.<br>2/2010 Lin et al.<br>4/2010 Inagaki et al.<br>5/2010 Lin et al.<br>11/2010 Stol et al.<br>12/2010 Kilmer et al.<br>10/2011 Morita et al.<br>3/2012 Kamat et al.<br>6/2012 Gejima<br>6/2014 Shibata<br>8/2014 Lin et al.<br>12/2014 Kamat et al.<br>12/2014 Kamat et al.<br>12/2014 Hosch et al.<br>1/2017 Wyatt-Mair et al.<br>1/2017 Wilhelmy et al.<br>3/2017 Boselli et al.<br>5/2017 Lin et al.<br>5/2017 Lin et al.<br>5/2017 Yan et al.<br>6/2017 Ahmed et al.<br>6/2017 Wen et al.<br>10/2017 Karabin et al.<br>10/2017 Lin et al.<br>10/2017 Lin et al.<br>10/2017 Lin et al.<br>10/2017 Lin et al.<br>10/2017 Lin et al.<br>11/2017 Go et al.<br>11/2017 Heard et al.<br>11/2017 Heard et al.<br>12/2017 Kang et al.<br>6/2018 Yan et al.<br>6/2018 Muller et al.<br>7/2018 Kilmer et al.<br>6/2019 Kilmer et al.<br>6/2019 Wilhelmy et al.<br>10/2019 Karabin et al.<br>11/2019 Kilmer et al.<br>2/2020 Heard et al.<br>3/2020 Ahmed et al.<br>4/2020 Boselli et al.<br>6/2020 Zehnder et al. |
| (51) | <b>Int. Cl.</b><br><i>C22C 21/10</i> (2006.01)<br><i>C22C 21/14</i> (2006.01)<br><i>C22C 21/16</i> (2006.01)<br><i>C22C 21/18</i> (2006.01)<br><i>C22F 1/043</i> (2006.01)<br><i>C22F 1/053</i> (2006.01)                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                               | 2008/0274367 A1<br>2010/0047113 A1<br>2010/0089503 A1<br>2010/0129683 A1<br>2010/0276108 A1<br>2010/0304175 A1<br>2011/0247736 A1<br>2012/0055590 A1<br>2012/0156089 A1<br>2014/0166165 A1<br>2014/0230974 A1<br>2014/0366997 A1<br>2014/0366998 A1<br>2014/0367000 A1<br>2015/0020930 A1<br>2015/0217599 A1<br>2016/0107265 A1<br>2016/0160333 A1<br>2017/0009325 A1<br>2017/0014937 A1<br>2017/0088920 A1<br>2017/0120386 A1<br>2017/0120393 A1<br>2017/0121795 A1<br>2017/0175239 A1<br>2017/0175240 A1<br>2017/0292174 A1<br>2017/0306447 A1<br>2017/0306448 A1<br>2017/0306449 A1<br>2017/0306450 A1<br>2017/0306457 A1<br>2017/0306460 A1<br>2017/0314112 A1<br>2017/0326690 A1<br>2017/0326868 A1<br>2017/0369978 A1<br>2018/0171438 A1<br>2018/0179621 A1<br>2018/0200834 A1<br>2019/0193149 A1<br>2019/0193158 A1<br>2019/0309402 A1<br>2019/0357647 A1<br>2020/0056268 A1<br>2020/0080182 A1<br>2020/0115780 A1<br>2020/0189314 A1                                                                                                                                      |                                                                                                                                                                                                                                                                                                                                                                                                                                                                                                                                                                                                                                                                                                                                                                                                                                                                                                                                                                                                                                                                                                                                                                                       |
| (52) | <b>U.S. Cl.</b><br>CPC ..... <i>C22C 21/16</i> (2013.01); <i>C22C 21/18</i> (2013.01); <i>C22F 1/043</i> (2013.01); <i>C22F 1/053</i> (2013.01)                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                         | 2012/0055590 A1<br>2012/0156089 A1<br>2014/0166165 A1<br>2014/0230974 A1<br>2014/0366997 A1<br>2014/0366998 A1<br>2014/0367000 A1<br>2015/0020930 A1<br>2015/0217599 A1<br>2016/0107265 A1<br>2016/0160333 A1<br>2017/0009325 A1<br>2017/0014937 A1<br>2017/0088920 A1<br>2017/0120386 A1<br>2017/0120393 A1<br>2017/0121795 A1<br>2017/0175239 A1<br>2017/0175240 A1<br>2017/0292174 A1<br>2017/0306447 A1<br>2017/0306448 A1<br>2017/0306449 A1<br>2017/0306450 A1<br>2017/0306457 A1<br>2017/0306460 A1<br>2017/0314112 A1<br>2017/0326690 A1<br>2017/0326868 A1<br>2017/0369978 A1<br>2018/0171438 A1<br>2018/0179621 A1<br>2018/0200834 A1<br>2019/0193149 A1<br>2019/0193158 A1<br>2019/0309402 A1<br>2019/0357647 A1<br>2020/0056268 A1<br>2020/0080182 A1<br>2020/0115780 A1<br>2020/0189314 A1                                                                                                                                                                                                                                                                           |                                                                                                                                                                                                                                                                                                                                                                                                                                                                                                                                                                                                                                                                                                                                                                                                                                                                                                                                                                                                                                                                                                                                                                                       |
| (58) | <b>Field of Classification Search</b><br>CPC ..... C22C 21/10; C22C 21/14; C22C 21/16; C22C 21/18                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                       | 2012/0055590 A1<br>2012/0156089 A1<br>2014/0166165 A1<br>2014/0230974 A1<br>2014/0366997 A1<br>2014/0366998 A1<br>2014/0367000 A1<br>2015/0020930 A1<br>2015/0217599 A1<br>2016/0107265 A1<br>2016/0160333 A1<br>2017/0009325 A1<br>2017/0014937 A1<br>2017/0088920 A1<br>2017/0120386 A1<br>2017/0120393 A1<br>2017/0121795 A1<br>2017/0175239 A1<br>2017/0175240 A1<br>2017/0292174 A1<br>2017/0306447 A1<br>2017/0306448 A1<br>2017/0306449 A1<br>2017/0306450 A1<br>2017/0306457 A1<br>2017/0306460 A1<br>2017/0314112 A1<br>2017/0326690 A1<br>2017/0326868 A1<br>2017/0369978 A1<br>2018/0171438 A1<br>2018/0179621 A1<br>2018/0200834 A1<br>2019/0193149 A1<br>2019/0193158 A1<br>2019/0309402 A1<br>2019/0357647 A1<br>2020/0056268 A1<br>2020/0080182 A1<br>2020/0115780 A1<br>2020/0189314 A1                                                                                                                                                                                                                                                                           |                                                                                                                                                                                                                                                                                                                                                                                                                                                                                                                                                                                                                                                                                                                                                                                                                                                                                                                                                                                                                                                                                                                                                                                       |
| (56) | <b>References Cited</b>                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                 |                                                                                                                                                                                                                                                                                                                                                                                                                                                                                                                                                                                                                                                                                                                                                                                                                                                                                                                                                                                                                                                                                   |                                                                                                                                                                                                                                                                                                                                                                                                                                                                                                                                                                                                                                                                                                                                                                                                                                                                                                                                                                                                                                                                                                                                                                                       |
|      | <b>U.S. PATENT DOCUMENTS</b>                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                            |                                                                                                                                                                                                                                                                                                                                                                                                                                                                                                                                                                                                                                                                                                                                                                                                                                                                                                                                                                                                                                                                                   |                                                                                                                                                                                                                                                                                                                                                                                                                                                                                                                                                                                                                                                                                                                                                                                                                                                                                                                                                                                                                                                                                                                                                                                       |
|      | 6,528,183 B2 3/2003 Dif et al.<br>6,555,251 B2 4/2003 Kilmer<br>6,705,384 B2 3/2004 Kilmer et al.<br>6,733,566 B1 5/2004 Fang et al.<br>6,773,666 B2 8/2004 Lin et al.<br>6,783,730 B2 8/2004 Lin et al.<br>6,925,711 B2 8/2005 Kilmer et al.<br>6,939,416 B2 9/2005 Benedictus et al.<br>7,087,125 B2 8/2006 Lin et al.<br>7,255,932 B1 8/2007 Kilmer<br>7,337,941 B2 3/2008 Scott et al.<br>7,374,827 B2 5/2008 Kilmer<br>7,449,073 B2 11/2008 Lin et al.<br>7,625,454 B2 12/2009 Lin et al.<br>7,732,059 B2 6/2010 Ren et al.<br>8,157,932 B2 4/2012 Yan et al.<br>8,273,196 B2 9/2012 Hibino et al.<br>8,287,668 B2 10/2012 Lin et al.<br>8,349,462 B2 1/2013 Lin et al.<br>8,366,846 B2 2/2013 Tataki et al.<br>8,840,737 B2 9/2014 Bray et al.<br>8,845,827 B2 9/2014 Yanai et al.<br>8,986,850 B2 3/2015 Baumann et al.<br>8,999,079 B2 4/2015 Kamat et al.<br>9,194,028 B2 11/2015 Kamat et al.<br>9,249,484 B2 2/2016 Kamat et al.<br>9,249,487 B2 2/2016 Yan et al.<br>9,315,885 B2 4/2016 Lin<br>9,359,660 B2 6/2016 Kamat et al.<br>9,458,528 B2 10/2016 Boselli et al.<br>9,587,298 B2 3/2017 Lin et al.<br>9,718,738 B2 8/2017 Iwig et al.<br>9,856,552 B2 1/2018 Sawtell et al.<br>9,890,443 B2 2/2018 Lin et al.<br>9,926,620 B2 3/2018 Kamat et al.<br>10,006,108 B2 6/2018 Wen et al.<br>10,119,183 B2 11/2018 Lin et al.<br>10,161,021 B2 12/2018 Lin et al.<br>10,174,409 B2 1/2019 Yan et al.<br>10,202,673 B2 2/2019 Lin et al.<br>10,227,679 B2 3/2019 Yan et al.<br>10,385,432 B2 8/2019 Kilmer et al.<br>10,494,702 B2 12/2019 Kim et al.<br>10,538,834 B2 1/2020 Wen et al.<br>10,589,327 B2 3/2020 Stewart et al.<br>10,704,128 B2 7/2020 Das et al.<br>11,103,919 B2 8/2021 Yan et al.<br>2003/0087122 A1 5/2003 Benedictus et al.<br>2004/0086417 A1 5/2004 Baumann et al. |                                                                                                                                                                                                                                                                                                                                                                                                                                                                                                                                                                                                                                                                                                                                                                                                                                                                                                                                                                                                                                                                                   |                                                                                                                                                                                                                                                                                                                                                                                                                                                                                                                                                                                                                                                                                                                                                                                                                                                                                                                                                                                                                                                                                                                                                                                       |
|      | <b>FOREIGN PATENT DOCUMENTS</b>                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                         |                                                                                                                                                                                                                                                                                                                                                                                                                                                                                                                                                                                                                                                                                                                                                                                                                                                                                                                                                                                                                                                                                   |                                                                                                                                                                                                                                                                                                                                                                                                                                                                                                                                                                                                                                                                                                                                                                                                                                                                                                                                                                                                                                                                                                                                                                                       |
|      | JP H11-310841 11/1999<br>JP 2001-020027 1/2001<br>JP 2001262264 9/2001<br>JP 2002-371333 12/2002<br>JP 2003-089859 3/2003<br>JP 2011-252212 12/2011<br>WO WO2005/075692 8/2005<br>WO WO-2015146654 A1 * 10/2015 ..... B21J 5/00<br>WO WO2018/157159 8/2018<br>WO WO2018/191111 10/2018<br>WO WO2018/048785 3/2019<br>WO WO2019/055623 3/2019<br>WO WO2019/055630 3/2019<br>WO WO2019/084045 5/2019                                                                                                                                                                                                                                                                                                                                                                                                                                                                                                                                                                                                                                                                                                                                                                                                                                                                                                                                                                                                                                                                                                                                                                                                                                                                                                                                                                                                      |                                                                                                                                                                                                                                                                                                                                                                                                                                                                                                                                                                                                                                                                                                                                                                                                                                                                                                                                                                                                                                                                                   |                                                                                                                                                                                                                                                                                                                                                                                                                                                                                                                                                                                                                                                                                                                                                                                                                                                                                                                                                                                                                                                                                                                                                                                       |
|      | <b>OTHER PUBLICATIONS</b>                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                               |                                                                                                                                                                                                                                                                                                                                                                                                                                                                                                                                                                                                                                                                                                                                                                                                                                                                                                                                                                                                                                                                                   |                                                                                                                                                                                                                                                                                                                                                                                                                                                                                                                                                                                                                                                                                                                                                                                                                                                                                                                                                                                                                                                                                                                                                                                       |
|      | WO2015146654A1, online machine translation (Year: 2015).*<br>JPH10219381A, online machine translation (Year: 1998).*                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                    |                                                                                                                                                                                                                                                                                                                                                                                                                                                                                                                                                                                                                                                                                                                                                                                                                                                                                                                                                                                                                                                                                   |                                                                                                                                                                                                                                                                                                                                                                                                                                                                                                                                                                                                                                                                                                                                                                                                                                                                                                                                                                                                                                                                                                                                                                                       |

(56)

**References Cited**

OTHER PUBLICATIONS

- ASTM F2792-12a, "Standard Terminology for Additive Manufacturing Technologies" ASTM International, 2014.
- ANSI H35.1, "American National Standard Alloy and Temper Designation Systems for Aluminum" The Aluminum Association Inc., 2009.
- International Search Report and Written Opinion, dated Feb. 15, 2019, from corresponding International Patent App. No. PCT/US2018/058421.
- Liang, W. J., et al., "General aspects related to the corrosion of 6xxx series aluminium alloys: exploring the influence of Mg/Si ratio and Cu" Corrosion Science 76:119-128, 2013.

\* cited by examiner



FIG. 1



FIG. 2

## ALUMINUM ALLOYS, AND METHODS FOR PRODUCING THE SAME

### CROSS-REFERENCE TO RELATED APPLICATION

This application is a continuation of International Patent Application No. PCT/US2018/058421, filed Oct. 31, 2018, which claims the benefit of priority of U.S. Patent Application No. 62/579,728, filed Oct. 31, 2017, and U.S. Patent Application No. 62/715,163, filed Aug. 6, 2018, each of which is incorporated herein by reference in its entirety.

### BACKGROUND

Aluminum alloys are useful in a variety of applications. However, improving one property of an aluminum alloy without degrading another property is elusive. For example, it is difficult to increase the strength of an alloy without decreasing the toughness of an alloy. Other properties of interest for aluminum alloys include corrosion resistance and fatigue resistance, to name two.

### SUMMARY OF THE DISCLOSURE

Broadly, the present patent application relates to new aluminum alloys, and methods for producing the same. Generally, the new aluminum alloy products are press-quenchable, where solution heat treatment after hot working is not required to achieve final properties. Thus, methods of producing the aluminum alloys may be absent of any solution heat treatment step after the final hot working step. As used herein, solution heat treatment includes quenching.

The new aluminum alloys may be produced in wrought form, such as an in rolled form (e.g., as sheet or plate), as an extrusion, or as a forging, among others. In one embodiment, the new aluminum alloy is in the form of a forged wheel product (e.g., a press-quenched forged wheel product). In one embodiment, the forged wheel product is a die-forged wheel product. In one embodiment, the new aluminum alloy is in the form of an extruded product (e.g., a press-quenched extruded product). In one embodiment, a new aluminum alloy product realizes a pitting only rating, or "P" rating, or better, when tested in accordance with ASTM G110. In one embodiment, a new aluminum alloy product has good intergranular (IG) corrosion resistance, realizing a maximum depth of attack of not greater than 500 microns when tested in accordance with ASTM G110.

#### I. Composition

The new aluminum alloys generally comprise (and some instances consist essentially of, or consist of) silicon (Si), magnesium (Mg), copper (Cu), zinc (Zn), and iron (Fe), optionally with one or more of manganese (Mn), chromium (Cr), vanadium (V), zirconium (Zr), and titanium (Ti), the balance being aluminum and impurities. The new aluminum alloys generally include Q phase precipitates, and the solvus temperature of these Q phase precipitates is generally not greater than 950° F.

The new aluminum alloys generally include from 0.6 to 1.4 wt. % Si, from 0.25 to 0.90 wt. % Mg, where the ratio of wt. % Si to wt. % Mg is from 1.05:1 to 5.0:1, from 0.25 to 2.0 wt. % Cu, from 0.10 to 3.5 wt. % Zn, and from 0.01 to 1.0 wt. % Fe. The new aluminum alloys may optionally include up to 0.8 wt. % Mn, up to 0.25 wt. % Cr, up to 0.20 wt. % Zr, up to 0.20 wt. % V, and up to 0.15 wt. % Ti. The total content of Fe+Mn+Cr+Zr+V+Ti within the new aluminum alloys is generally not greater than 2.0 wt. %.

As noted above, the new aluminum alloys generally include silicon and in the range of from 0.60 wt. % to 1.4 wt. % Si. In one embodiment, a new aluminum alloy includes at least 0.65 wt. % silicon. In one embodiment, a new aluminum alloy includes not greater than 1.35 wt. % silicon. In another embodiment, a new aluminum alloy includes not greater than 1.3 wt. % silicon.

As noted above, the new aluminum alloys generally include magnesium and in the range of from 0.25 to 0.90 wt. % Mg. In one embodiment, a new aluminum alloy includes at least 0.30 wt. % Mg. In another embodiment, a new aluminum alloy includes at least 0.35 wt. % Mg. In yet another embodiment, a new aluminum alloy includes at least 0.40 wt. % Mg. In another embodiment, a new aluminum alloy includes at least 0.45 wt. % Mg.

As noted above, the new aluminum alloys generally have a ratio of wt. % Si to wt. % Mg of from 1.05:1 to 5.0:1 (Si:Mg). In one embodiment, the ratio of wt. % Si to wt. % Mg is from 1.05:1 to 4.67:1. In another embodiment, the ratio of wt. % Si to wt. % Mg is from 1.05:1 to 4.0:1. In yet another embodiment, the ratio of wt. % Si to wt. % Mg is from 1.05:1 to 3.5:1. In another embodiment, the ratio of wt. % Si to wt. % Mg is from 1.05:1 to 3.1:1. In one embodiment, the ratio of wt. % Si to wt. % Mg is not greater than 2.75:1. In another embodiment, the ratio of wt. % Si to wt. % Mg is not greater than 2.5:1. In one embodiment, the ratio of wt. % Si to wt. % Mg is at least 1.10:1. In another embodiment, the ratio of wt. % Si to wt. % Mg is at least 1.25:1. In yet another embodiment, the ratio of wt. % Si to wt. % Mg is at least 1.50:1. In another embodiment, the ratio of wt. % Si to wt. % Mg is at least 1.75:1.

As noted above, the new aluminum alloys generally include from 0.25 to 2.0 wt. % Cu. In one embodiment, a new aluminum alloy includes an amount of copper sufficient such that an aluminum alloy product realizes a pitting only rating, or "P" rating, when tested in accordance with ASTM G110. In one embodiment, a new aluminum alloy includes an amount of copper sufficient such that an aluminum alloy product realizes a maximum depth of attack of not greater than 500 micrometers when tested in accordance with ASTM G110. In another embodiment, a new aluminum alloy includes an amount of copper sufficient such that an aluminum alloy product realizes a maximum depth of attack of not greater than 250 micrometers when tested in accordance with ASTM G110. In one embodiment, a new aluminum alloy includes at least 0.30 wt. % Cu. In another embodiment, a new aluminum alloy includes at least 0.50 wt. % Cu. In yet another embodiment, a new aluminum alloy includes at least 0.75 wt. % Cu. In yet another embodiment, a new aluminum alloy includes at least 1.0 wt. % Cu. In one embodiment, a new aluminum alloy includes not greater than 1.75 wt. % Cu. In another embodiment, a new aluminum alloy includes not greater than 1.5 wt. % Cu.

As noted above, the new aluminum alloys generally include from 0.10 to 3.5 wt. % Zn. Zinc may be used for solid solution strengthening. In one embodiment, a new aluminum alloy includes an amount of zinc sufficient such that an aluminum alloy product realizes a pitting only rating, or "P" rating, when tested in accordance with ASTM G110. In one embodiment, a new aluminum alloy includes an amount of zinc sufficient such that an aluminum alloy product realizes a maximum depth of attack of not greater than 500 micrometers when tested in accordance with ASTM G110. In another embodiment, a new aluminum alloy includes an amount of zinc sufficient such that an aluminum alloy product realizes a maximum depth of attack of not greater than 250 micrometers when tested in accordance with ASTM G110.

dance with ASTM G110. In one embodiment, a new aluminum alloy includes at least 0.20 wt. % Zn. In another embodiment, a new aluminum alloy includes at least 0.30 wt. % Zn. In yet another embodiment, a new aluminum alloy includes at least 0.50 wt. % Zn. In one embodiment, a new aluminum alloy includes not greater than 3.0 wt. % Zn. In another embodiment, a new aluminum alloy includes not greater than 2.5 wt. % Zn.

As noted above, the new aluminum alloys generally include from 0.01 to 1.0 wt. % Fe. Iron may help facilitate the appropriate amounts and/or types of intermetallic particles of the aluminum alloy. In one embodiment, a new aluminum alloy includes at least 0.03 wt. % Fe. In another embodiment, a new aluminum alloy includes at least 0.06 wt. % Fe. In yet another embodiment, a new aluminum alloy includes at least 0.09 wt. % Fe. In another embodiment, a new aluminum alloy includes at least 0.12 wt. % Fe. In yet another embodiment, a new aluminum alloy includes at least 0.15 wt. % Fe. In one embodiment, a new aluminum alloy includes not greater than 0.75 wt. % Fe. In another embodiment, a new aluminum alloy includes not greater than 0.60 wt. % Fe. In yet another embodiment, a new aluminum alloy includes not greater than 0.50 wt. % Fe. In another embodiment, a new aluminum alloy includes not greater than 0.40 wt. % Fe. In yet another embodiment, a new aluminum alloy includes not greater than 0.30 wt. % Fe. In another embodiment, a new aluminum alloy includes not greater than 0.25 wt. % Fe. In yet another embodiment, a new aluminum alloy includes not greater than 0.22 wt. % Fe.

As noted above, the new aluminum alloys may include up to 0.80 wt. % Mn. In one embodiment, a new aluminum alloy includes at least 0.05 wt. % Mn. In another embodiment, a new aluminum alloy includes at least 0.08 wt. % Mn. In yet another embodiment, a new aluminum alloy includes at least 0.10 wt. % Mn. In one embodiment, a new aluminum alloy includes not greater than 0.70 wt. % Mn. In another embodiment, a new aluminum alloy includes not greater than 0.60 wt. % Mn. In yet another embodiment, a new aluminum alloy includes not greater than 0.50 wt. % Mn. In another embodiment, a new aluminum alloy includes not greater than 0.40 wt. % Mn. In yet another embodiment, a new aluminum alloy includes not greater than 0.30 wt. % Mn. In another embodiment, a new aluminum alloy includes not greater than 0.25 wt. % Mn. In yet another embodiment, a new aluminum alloy includes not greater than 0.20 wt. % Mn. In another embodiment, a new aluminum alloy includes not greater than 0.18 wt. % Mn.

As noted above, the new aluminum alloys may include up to 0.25 wt. % Cr. In one embodiment, a new aluminum alloy includes at least 0.05 wt. % Cr. In another embodiment, a new aluminum alloy includes at least 0.08 wt. % Cr. In yet another embodiment, a new aluminum alloy includes at least 0.12 wt. % Cr. In another embodiment, a new aluminum alloy includes at least 0.15 wt. % Cr. In yet another embodiment, a new aluminum alloy includes at least 0.18 wt. % Cr. In one embodiment, a new aluminum alloy includes not greater than 0.22 wt. % Cr.

As noted above, the new aluminum alloys may include up to 0.20 wt. % Zr. In one embodiment, a new aluminum alloy includes not greater than 0.05 wt. % Zr. In another embodiment, a new aluminum alloy includes not greater than 0.03 wt. % Zr. In yet another embodiment, a new aluminum alloy includes not greater than 0.01 wt. % Zr.

As noted above, the new aluminum alloys may include up to 0.20 wt. % V. In one embodiment, a new aluminum alloy includes not greater than 0.05 wt. % V. In another embodiment, a new aluminum alloy includes not greater than 0.03

wt. % V. In yet another embodiment, a new aluminum alloy includes not greater than 0.01 wt. % V.

As noted above, the new aluminum alloys may include up to 0.15 wt. % Ti. In one embodiment, a new aluminum alloy includes at least 0.01 wt. % Ti. In another embodiment, a new aluminum alloy includes at least 0.02 wt. % Ti.

As noted above, the new aluminum alloys generally include a total of Fe+Mn+Cr+Zr+V+Ti of not greater than 2.0 wt. %. In one embodiment, a new aluminum alloy includes a total of Fe+Mn+Cr+Zr+V+Ti of not greater than 1.75 wt. %. In another embodiment, a new aluminum alloy includes a total of Fe+Mn+Cr+Zr+V+Ti of not greater than 1.50 wt. %. In yet another embodiment, a new aluminum alloy includes a total of Fe+Mn+Cr+Zr+V+Ti of not greater than 1.25 wt. %. In another embodiment, a new aluminum alloy includes a total of Fe+Mn+Cr+Zr+V+Ti of not greater than 1.0 wt. %. In one embodiment, a new aluminum alloy includes a total of Fe+Mn+Cr+Zr+V+Ti of not greater than 0.8 wt. %. In another embodiment, a new aluminum alloy includes a total of Fe+Mn+Cr+Zr+V+Ti of not greater than 0.65 wt. %.

As noted above, the new aluminum alloys generally include at least some Q phase precipitates (Al—Cu—Mg—Si style precipitates, such as Al<sub>5</sub>Cu<sub>2</sub>Mg<sub>8</sub>Si<sub>6</sub>), and the solvus temperature of these Q phase precipitates is not greater than 950° F. In one embodiment, the Q phase precipitates realize a solvus temperature of not greater than 925° C. In another embodiment, the Q phase precipitates realize a solvus temperature of not greater than 900° F. In yet another embodiment, the Q phase precipitates realize a solvus temperature of not greater than 875° F. In another embodiment, the Q phase precipitates realize a solvus temperature of not greater than 850° F. In yet another embodiment, the Q phase precipitates realize a solvus temperature of not greater than 825° F.

In addition to the Q phase precipitates, the new aluminum alloys may include Mg<sub>2</sub>Si precipitates. When a new aluminum alloy includes Mg<sub>2</sub>Si precipitates, generally the volumetric ratio of Mg<sub>2</sub>Si precipitates to Q phase precipitates is not greater than 1.25:1 (Mg<sub>2</sub>Si:Q phase). In one embodiment, the volumetric ratio of Mg<sub>2</sub>Si precipitates to Q phase precipitates is not greater than 1.10:1. In another embodiment, the volumetric ratio of Mg<sub>2</sub>Si precipitates to Q phase precipitates is not greater than 1.05:1. In yet another embodiment, the volumetric ratio of Mg<sub>2</sub>Si precipitates to Q phase precipitates is not greater than 1.0:1. In yet another embodiment, the volumetric ratio of Mg<sub>2</sub>Si precipitates to Q phase precipitates is less than 1:0:1. In another embodiment, the volumetric ratio of Mg<sub>2</sub>Si precipitates to Q phase precipitates is not greater than 0.95:1. In any of these embodiments the Mg<sub>2</sub>Si precipitates may realize a solvus temperature of not greater than 950° F.

In one embodiment, a new aluminum alloy is essentially free of Al<sub>2</sub>Cu precipitates. In one embodiment, a new aluminum alloy is essentially free of Mg<sub>2</sub>Si precipitates. In one embodiment, a new aluminum alloy is essentially free of both Al<sub>2</sub>Cu precipitates and Mg<sub>2</sub>Si precipitates.

## II. Processing

As noted above, the new aluminum alloy may be processed to any wrought product form, including sheet, plate, forgings, or extrusions. The new aluminum alloy may also be shape cast, or may be used in additive manufacturing to produce an additively manufactured product. Additive manufacturing is defined in ASTM F2792-12a.

In one approach, a new aluminum alloy is made into a press-quenched product/is processed by press-quenching. As noted above, press-quenching generally involves hot

working a heat-treatable aluminum alloy into an intermediate or final product form, after which the method is free of any subsequent solution heat treatment. For purposes of this patent application, press-quenching includes isothermal forging.

in one embodiment, and referring now to FIG. 1, a method may comprise (a) preparing a new aluminum alloy for press-quenching (100), then (b) press-quenching the new aluminum alloy (200), thereby producing a press-quenched aluminum alloy product, and then (c) aging the press-quenched aluminum alloy product (300). In these embodiments of FIG. 1, after the press-quenching step (b), the method is absent of any solution heat treatment step. Cold working (400) may optionally be completed after the press quenching step (200).

Regarding the preparing for press-quenching step (100), the method may include the steps of (i) producing an ingot or billet of the new aluminum alloy and (ii) homogenizing the ingot or billet. The homogenization can include one or multiple soak temperatures. The preparing step (100) may also include some hot working and/or cold working, in some circumstances.

Regarding the press-quenching step (200), the method may include (i) working (210) (e.g. hot working) of the aluminum alloy (e.g., in the form of an ingot, a billet, or a prior worked product) into an intermediate or final product form, and (ii) after the working step, quenching the product form with a fluid (220), thereby producing a press-quenched aluminum alloy product. Regarding the working step (b)(i), the working may include using one or more workpieces (e.g., dies, molds, or rolls) to form the aluminum alloy into the product form. In one embodiment, the working step (210) produces the final product form (e.g., when no cold working (400) is applied after the press-quenching step (200)), and thus, after, the press-quenching (200), the press-quenched product is a final press-quenched product. In another embodiment, the working step (210) produces an intermediate product form (e.g., when cold working (400) is applied after the press-quenching step (200)), and thus, after, the press-quenching (200), the press-quenched product is an intermediate press-quenched product.

In one embodiment, prior to the working step (210), a starting working temperature of the aluminum alloy is above the solvus temperature of precipitates phases of the aluminum alloy. In another embodiment, prior to the working, a starting working temperature of the aluminum alloy is not greater than 1075° F., or not greater than 1050° F., or not greater than 1025° F., or not greater than 1000° F., or not greater than 975° F. In one embodiment, prior to the working, a starting working temperature of the aluminum alloy is both (I) above the solvus temperature of precipitates phases of the aluminum alloy, and (II) not greater than 1075° F., or not greater than 1050° F., or 1025° F., or not greater than 1000° F., or not greater than 975° F. After the working step, an ending working temperature of the product form (i.e., the temperature of the product immediately upon conclusion of the working step (210)) may be (I) above the solvus temperature of the precipitates phases of the aluminum alloy, or (II) below the solvus temperature of the precipitate phases but within 100° F. of the solvus temperature of the precipitates phases of the aluminum alloy. In one embodiment, the working comprises extruding. In another embodiment, the working comprises forging. In one embodiment, the working comprises rotary forging. In one embodiment, the working comprises rolling. In one embodiment, the working

comprises isothermally working (e.g., isothermally forging). In another embodiment, the working comprises non-isothermally working.

Regarding the quenching step (220), the quenching may 5 comprise cooling the product form from the working temperature to below 600° F. and at a quench rate of at least 5° F. per second. In one embodiment, the quench rate is at least 10° F. per second. In another embodiment, the quench rate is at least 20° F. per second. In yet another embodiment, the quench rate is at least 50° F. per second. In another embodiment, the quench rate is at least 100° F. per second.

The quenching (220) generally comprises contacting the worked product with a quenching medium. The quenching medium may be any suitable gas, liquid, or combination 15 thereof. In one embodiment, the quenching medium comprises a liquid. In one embodiment, the quenching medium comprises a gas. In one embodiment, the quenching medium is air. In one embodiment, the quenching comprises at least 20 one of: (I) immersion of the product form in a liquid and (II) spraying of the product form with a liquid (e.g., spraying of water) or gas (e.g., blowing of air).

Regarding the aging step (300), the aging may include naturally aging to a substantially stable condition (per ANSI 25 H35.1) or artificially aging the press-quenched aluminum alloy product. The artificial aging may comprise single step aging processes or multiple step aging processes. The artificial aging may be underaging, peak aging (e.g., within 2 ksi of peak strength), or overaging.

Products that are press-quenched and then only naturally 30 aged are generally in a T1 temper. Products that are press-quenched and then only artificially aged are generally in a T5 temper. Products that are press-quenched, and then cold worked and then naturally aged are in a T2 temper. Products that are press-quenched, and then cold worked and then 35 artificially aged are in a T10 temper. The new aluminum alloys described herein may be produced in any of a T1, T2 T5 or T10 temper. Thus, in some embodiments, the press-quenched aluminum alloy product is in one of a T1, T2, T5 or T10 temper, as per ANSI H35.1 (2009).

In one embodiment, the aging (300) is natural aging to a 40 substantially stable condition, as per ANSI H35.1 (2009). In one embodiment, the aging (300) comprises artificial aging. In one embodiment, the method is absent of any cold working step (400) after the press-quenching step (b). In another embodiment, cold working (400) is performed after the press-quenching step (b), i.e., the product is in either a T2 or a T10 temper, as per ANSI H35.1 (2009). The cold working may reduce the thickness of the press-quenched product by any appropriate amount, such as by cold working 45 to achieve a reduction in thickness of from 10-75%. In one embodiment, the cold working (400) achieves a reduction in thickness of from 10-50%. The cold working (400) may be accomplished by one or more of rolling, extruding, forging, drawing, ironing, spinning, flow-forming, and combinations 50 thereof, among other types of cold working methods.

The new aluminum alloys may also be made without 55 press-quenching. In one embodiment, a new aluminum alloy is made into one of a T3, T4, T6, T7, T8 or T9 temper, as per ANSI H35.1. For instance, and with reference now to FIG. 60 2, a method may include (a) preparing a new aluminum alloy for solution heat treatment (500), (b) solution heat treating the aluminum alloy (600), and (c) aging the aluminum alloy (300). Cold working (400) may optionally be completed after the solution heat treating step (600).

The preparing step (500) may be generally similar to the preparing step (100) of FIG. 1, and may include producing an ingot or billet of the new aluminum alloy and then

homogenizing the ingot or billet (510). The homogenization (510) can include one or multiple soak temperatures. The preparing step (500) generally includes working (520) of the ingot or billet into an intermediate or final product form. The working (520) generally includes hot working, optionally with cold working. Annealing may optionally be used after any cold working step, but annealing is often not required. Any annealing occurs before the solution heat treating (600).

After the preparing step (500), the worked aluminum alloy product is generally solution heat treated (600). The solution heat treatment (600) may include heating the worked aluminum alloy product to one or more suitable soak temperatures, generally above the solvus temperature, holding at this/these temperature(s) long enough to allow soluble elements to enter into solid solution, and then cooling rapidly enough to hold the elements in solid solution. The heating may be accomplished, for example, via a suitable furnace. No working is completed during the solution heat treating step (600). The subsequent quenching may be completed, for instance, by exposure to an appropriate quenching medium, such as by immersion, spraying and/or jet drying, among other techniques, as described above relative to press-quenching step (200).

After the solution heat treating (600), the aluminum alloy product may be naturally aged or artificially aged (300), and as described above relative to FIG. 1.

For products to be produced in the T4 temper, the solution heat treated product is naturally aged, but without further working (i.e., no hot working or cold working is completed after the solution heat treatment), or artificially aging.

For products to be produced in the T6 or T7 temper, the solution heat treated product is artificially aged after solution heat treatment and without any further working (i.e., no hot working or cold working is completed after the solution heat treatment or after the artificial aging).

For products to be produced in the T9 temper, the solution heat treated product is first artificially aged and then cold worked (not shown in FIG. 2).

For products to be produced in the T3 temper, the aluminum alloy product is cold worked after solution heat treatment, and then naturally aged (but not artificially aged).

For products to be produced in the T8 temper, the aluminum alloy product is cold worked after solution heat treatment, and then artificially aged.

For the T3 and T8 temper products, the post-solution heat treatment working generally results in the aluminum alloy product being in its final form/final gauge prior to the natural or artificial aging. For the T9 temper products, the post-artificial aging working results in the aluminum alloy product being in its final form/final gauge.

For shape castings and additively manufactured products, the preparing step (500) is optional, i.e., such products may only include the solution heat treating (600) and aging (300) steps. However, shape castings and additively manufactured products can also be worked, if useful, and such working can be completed pre-solution heat treatment, post-solution heat treatment, or both. Shape castings and additively manufactured products can also be press-quenched, if useful. For purposes of this patent application, shape castings also includes products made by semi-solid metal casting processes, such as squeeze casting.

### III. Applications

As noted above, the new aluminum alloys may be produced in wrought form, such as an in rolled form (e.g., as sheet or plate), as an extrusion, or as a forging, among others. The new aluminum alloy may also be in the form of a shape cast product or an additively manufactured product.

Such wrought, shape-cast, or additively manufactured products may be used in a variety of applications. In one embodiment, a new aluminum alloy product is in the form of a wheel product (e.g., shape-cast or forged wheel product or a press-quenched forged wheel product). In one embodiment, a forged wheel product is a die-forged wheel product. In one embodiment, a wheel product is a commercial truck wheel product (e.g., for light, medium or heavy-duty applications for trucks, buses or trailers). In one embodiment, a new aluminum alloy product is used as an automotive component, such as a closure panel, a body-in-white (BIW) structure (e.g., A, B or C pillars), a drive-shaft, or a suspension component, among others. In one embodiment, the automotive component is an energy absorbing component (e.g., a bumper, a shock tower). Pipe, fuel cylinders and core barrels (drill pipe), for instance, may also be produced from the new aluminum alloys. Other known product applications for aluminum alloys may also be employed.

### BRIEF DESCRIPTION OF THE DRAWINGS

FIG. 1 is a flow chart illustrating various methods for producing press-quenched aluminum alloy products

FIG. 2 is a flow chart illustrating various method for producing solution heat treated aluminum alloy products.

### DETAILED DESCRIPTION

#### Example 1

Fourteen alloys were modeled using PANDAT thermodynamic modeling software. The compositions of the fourteen alloys are given in Table 1, below. Alloy 1-7 are invention alloys. The other alloys are conventional aluminum alloys.

TABLE 1

| Alloy | Composition of Modeled Alloys (in wt. %) |      |      |      |      |       |      |        | Si +<br>Mg |
|-------|------------------------------------------|------|------|------|------|-------|------|--------|------------|
|       | Si                                       | Mg   | Cu   | Zn   | Fe   | Mn    | Cr   | Si:Mg  |            |
| 1     | 0.9                                      | 0.48 | 0.6  | 0.72 | 0.2  | 0.15  | 0.2  | 1.88:1 | 1.38       |
| 2     | 0.9                                      | 0.48 | 0.6  | 3.0  | 0.2  | 0.15  | 0.2  | 1.88:1 | 1.38       |
| 3     | 0.7                                      | 0.61 | 0.6  | 2.0  | 0.15 | 0.1   | 0    | 1.15:1 | 1.31       |
| 4     | 1.3                                      | 0.61 | 0.6  | 2.0  | 0.15 | 0.1   | 0    | 2.13:1 | 1.91       |
| 5     | 0.9                                      | 0.48 | 0.9  | 1.0  | 0.2  | 0.15  | 0.2  | 1.88:1 | 1.38       |
| 6     | 0.9                                      | 0.48 | 0.3  | 2.0  | 0.2  | 0.15  | 0.2  | 1.88:1 | 1.38       |
| 7     | 0.8                                      | 0.7  | 0.9  | 2.0  | 0.2  | 0.15  | 0.2  | 1.14:1 | 1.5        |
| 8     | 1.1                                      | 0.55 | 1.2  | 0.5  | 0.2  | 0.14  | 0.2  | 2.0:1  | 1.65       |
| 9     | 1.1                                      | 0.55 | 1.5  | 0.2  | 0.2  | 0.14  | 0.2  | 2.0:1  | 1.65       |
| 10    | 1.1                                      | 0.55 | 1.8  | 0.2  | 0.2  | 0.14  | 0.2  | 2.0:1  | 1.65       |
| 6061  | 0.69                                     | 0.9  | 0.9  | 0    | 0.2  | 0.075 | 0.2  | 0.77:1 | 1.59       |
| 6361  | 0.75                                     | 1.2  | 1.2  | 0    | 0.15 | 0.14  | 0.24 | 0.63:1 | 1.95       |
| 6056  | 1.0                                      | 0.9  | 0.9  | 0.4  | 0.25 | 0.7   | 0.25 | 1.11:1 | 1.9        |
| 6156  | 1.0                                      | 0.95 | 0.95 | 0.4  | 0.15 | 0.55  | 0.25 | 1.05:1 | 1.95       |
| 6013  | 0.75                                     | 0.95 | 0.95 | 0    | 0.15 | 0.35  | 0.08 | 0.79:1 | 1.7        |
| 6055  | 0.9                                      | 0.9  | 0.9  | 0.72 | 0.1  | 0.08  | 0.24 | 1:1    | 1.8        |
| 6099  | 1.0                                      | 0.95 | 0.95 | 0.8  | 0.15 | 0.25  | 0.2  | 1.05:1 | 1.95       |

Table 2, below, includes the modeled thermodynamic properties of the alloys.

TABLE 2

## Thermodynamic Properties of Modeled Alloys

| Alloy | Liquidus<br>(° F.) | Solidus<br>(° F.) | Mg <sub>2</sub> Si<br>Solvus<br>(° F.) | Q-phase<br>solvus<br>(° F.) | Amount of<br>precipitates<br>at 390° F.<br>(mol. %) | Precipitate<br>Phases                       |
|-------|--------------------|-------------------|----------------------------------------|-----------------------------|-----------------------------------------------------|---------------------------------------------|
| 1     | 1202               | 1084              | 877                                    | 811                         | 1.63                                                | Q + Si                                      |
| 2     | 1194               | 1055              | 870                                    | 818                         | 1.68                                                | Q + Si                                      |
| 3     | 1197               | 1078              | 933                                    | 815                         | 1.86                                                | Q + Si                                      |
| 4     | 1191               | 1014              | 918                                    | 839                         | 2.44                                                | Q + Si                                      |
| 5     | 1199               | 1070              | —                                      | 884                         | 1.64                                                | Q + Si                                      |
| 6     | 1199               | 1078              | 871                                    | 734                         | 1.61                                                | Q + Si + Mg <sub>2</sub> Si                 |
| 7     | 1197               | 1066              | 950                                    | 822                         | 1.88                                                | Q + Mg <sub>2</sub> Si                      |
| 8     | 1197               | 1044              | —                                      | 913                         | 1.98                                                | Q + Si                                      |
| 9     | 1197               | 1037              | —                                      | 924                         | 2.78                                                | Q + Si + Al <sub>2</sub> Cu                 |
| 10    | 1195               | 1025              | —                                      | 935                         | 3.18                                                | Q + Al <sub>2</sub> Cu                      |
| 6061  | 1204               | 1105              | 964                                    | —                           | 1.79                                                | Mg <sub>2</sub> Si + Al <sub>2</sub> Cu     |
| 6361  | 1212               | 1080              | 1010                                   | —                           | 2.36                                                | Mg <sub>2</sub> Si + Al <sub>2</sub> Cu     |
| 6056  | 1210               | 1050              | 1005                                   | 865                         | 2.65                                                | Q + Mg <sub>2</sub> Si                      |
| 6156  | 1210               | 1046              | 1005                                   | 879                         | 2.5                                                 | Q + Mg <sub>2</sub> Si                      |
| 6013  | 1199               | 1071              | 996                                    | 829                         | 2.75                                                | Mg <sub>2</sub> Si + Al <sub>2</sub> Cu + Q |
| 6055  | 1207               | 1053              | 1000                                   | 851                         | 2.32                                                | Q + Mg <sub>2</sub> Si                      |
| 6099  | 1200               | 1064              | 1015                                   | 781                         | 2.33                                                | Q + Mg <sub>2</sub> Si                      |

As shown, the inventive alloys realize Q phase precipitates and these precipitates have low solvus temperatures, indicating applicability to press-quenching. Further, many are free of Al<sub>2</sub>Cu and Mg<sub>2</sub>Si precipitates.

While various embodiments of the new technology described herein have been described in detail, it is apparent that modifications and adaptations of those embodiments will occur to those skilled in the art. However, it is to be expressly understood that such modifications and adaptations are within the spirit and scope of the presently disclosed technology.

What is claimed is:

1. An aluminum alloy comprising:

0.6-1.4 wt. % Si;

0.25-0.90 wt. % Mg;

wherein the ratio of wt. % Si to wt. % Mg is from 1.05:1 to 5.0:1;

0.25-2.0 wt. % Cu;

0.10-3.5 wt. % Zn;

0.01-1.0 wt. % Fe;

up to 0.8 wt. % Mn;

up to 0.25 wt. % Cr;

up to 0.20 wt. % Zr;

up to 0.20 wt. % V;

up to 0.15 wt. % Ti;

wherein the total of Fe+Mn+Cr+Zr+V+Ti is not greater than 2.0 wt. %;

the balance being aluminum and impurities;

wherein the aluminum alloy includes Q phase precipitates; and

wherein the solvus temperature of the Q phase precipitates and any Mg<sub>2</sub>Si precipitates is not greater than 950° F.

2. The aluminum alloy of claim 1, wherein the aluminum alloy includes at least 0.7 wt. % Si.

3. The aluminum alloy of claim 2, wherein the aluminum alloy includes not greater than 1.3 wt. % Si.

4. The aluminum alloy of claim 1, wherein the aluminum alloy includes at least 0.30 wt. % Mg, and wherein the ratio of wt. % Si to wt. % Mg is from 1.05:1 to 4.67:1.

5. The aluminum alloy of claim 4, wherein the ratio of wt. % Si to wt. % Mg is at least 1.10:1.

6. The aluminum alloy of claim 5, wherein the ratio of wt. % Si to wt. % Mg is not greater than 2.75:1, or not greater than 2.5:1.

7. The aluminum alloy of claim 1, wherein the aluminum alloy includes at least 0.30 wt. % Cu.

8. The aluminum alloy of claim 7, wherein the aluminum alloy includes not greater than 1.75 wt. % Cu.

9. The aluminum alloy of claim 1, wherein the aluminum alloy includes at least 0.20 wt. % Zn.

10. The aluminum alloy of claim 9, wherein the aluminum alloy includes not greater than 3.0 wt. % Zn.

11. The aluminum alloy of claim 1, wherein the aluminum alloy includes from 0.10 to 0.30 wt. % Mn.

12. The aluminum alloy of claim 11, wherein the aluminum alloy includes not greater than 0.05 wt. % Zr and not greater than 0.05 wt. % V.

13. The aluminum alloy of claim 1, wherein the aluminum alloy includes the Q phase precipitates and Mg<sub>2</sub>Si precipitates, and a volumetric ratio of Mg<sub>2</sub>Si precipitates to Q phase precipitates is not greater than 1.25:1 ((Mg<sub>2</sub>Si(vol.)):(Q phase (vol.))).

\* \* \* \* \*